

## UNITED STATES PATENT OFFICE

2,238,850

MILDEWPROOFING AND MOTHPROOFING  
TREATMENT

Martin Leatherman, Hyattsville, Md.

No Drawing. Application November 23, 1938,  
Serial No. 242,124

4 Claims. (Cl. 21—6)

(Granted under the act of March 3, 1883, as  
amended April 30, 1928; 370 O. G. 757)

This application is made under the act of March 3, 1883, as amended by the act of April 30, 1928, and the invention herein described and claimed, if patented, may be manufactured and used by or for the Government of the United States of America for governmental purposes without the payment to me of any royalty thereon.

This invention relates to mildewproofing of cellulose fabrics which are used in contiguity with rubber, such as cotton hose lined with rubber, beltings, raincoats, rubberized shower curtains, rubber elasticized fabrics, and so forth. This invention also relates to a combination of mildewproofing and mothproofing for plant and animal fibre fabrics subject to the destructive action of fungi or insect larvae, such as wool, cotton, silk, mohair, and so forth.

One of the objects of this invention is to provide mildewproofing means which are colorless and which will not be readily removed by the ordinary so-called dry cleaning solvents or by water.

Heretofore, copper has been the most common mildewproofing metal, but it is unsatisfactory when used in rubberized fabrics because it induces changes in the rubber component and also the copper is absorbed by the rubber which destroys its mildewproofing action. I have discovered that cadmium has no injurious effect whatever upon rubber, and that it is approximately twice as effective as copper in inhibiting growth activity of organisms in cellulose.

I have also found that the common fatty acid soaps of cadmium such as the oleate, palmitate, and stearate are practically insoluble in such solvents as carbon tetrachloride, gasoline, Stoddards solvent, and solvent naphtha. This is not true with respect to the non-fatty acid soaps, such as the resinate which is very soluble in these solvents. For this reason, fabrics treated with the fatty acid soaps of cadmium may be dry cleaned, whereas the non-fatty acid soaps of cadmium would be removed from fabrics by dry cleaning.

I have found that five-hundredths of one percent of cadmium by weight is sufficient to prevent mildew of cellulose fabrics. An illustrative method of treating the fabric in accordance with my invention comprises saturating the fabric with a solution of ordinary alkali soap of sufficient concentration to fix approximately five-hundredths of one per cent of cadmium by weight, thence drying the fabric, and then immersing it in a solution of a cadmium salt as a

precipitant, such as the chloride, which solution preferably contains a wetting agent, such as sodium lauryl sulphate, for example. The fabric is then washed. If desired, it may also be treated with a solution to precipitate the wetting agent. When using sodium lauryl sulphate as the wetting agent, a solution of a potassium salt may be used for this purpose. The fabric is then dried. By treating the fabric, before the first drying step in the above-described method is completed, to obtain maximum absorbency, with a solution of cadmium silicofluoride both mildewproofing and mothproofing is effected and the remaining steps in the process may be omitted, since this solution precipitates the cadmium soap in the fabric. The fabric being somewhat damp, it absorbs sufficient cadmium fluosilicate solution to precipitate the soap compound, leaving a residue of cadmium soap and alkali fluosilicate in the fabric. Fluosilicates are of value for mothproofing, and the waterproofing effect of the cadmium soap prevents easy removal of the residual water-soluble cadmium and alkali fluosilicate except by prolonged exposure to water.

The cadmium soap may also be introduced into the fibrous material by making use of certain mixed solvents to dissolve the soap and carry it into and through the fibrous material. For example, the cadmium soap can be dissolved in a hot solution of a solvent consisting of two parts benzene, one part acetone, and one part methanol by volume. Mixed solvents, such as this one, especially when warm would retain enough cadmium soap in solution to permit the introduction of the soap into the material to be treated by wetting it with the solution and then drying the fabric.

Cadmium fluosilicate may also be used by itself to effect a combination of mildewproofing and mothproofing. Being soluble in water, but not in organic solvents, it may be employed in the home to temporarily protect washable garments which may be stored. Such garments can be treated by simply immersing them in the cadmium fluosilicate solution and then permitting the solvent to evaporate. So-called dry cleaning would not affect the fabric treated in this manner. A one-tenth of one percent solution of cadmium fluosilicate will normally introduce a sufficient protective quantity in the fabric after the fabric is wetted with it and squeezed, wrung, or centrifuged. Ordinarily, five-hundredths of one per cent by weight of elemental cadmium and an equal amount of the fluosilicate (SiF<sub>6</sub><sup>2-</sup>) radical will give satisfactory protection.

Having thus described my invention, I claim:

1. An article of manufacture comprising a rubberized cellulose fabric impregnated with a mildewproofing agent compatible with rubber, said agent containing a fatty acid soap of cadmium as its essential active ingredient.
2. An article of manufacture comprising a rubberized cellulose fabric impregnated with a mildewproofing agent compatible with rubber, said agent containing cadmium oleate as its essential 10 active ingredient.
3. An article of manufacture comprising a rub-

berized cellulose fabric impregnated with a mildewproofing agent compatible with rubber, said agent containing cadmium palmitate as its essential active ingredient.

- 5 4. An article of manufacture comprising a rubberized cellulose fabric impregnated with a mildewproofing agent compatible with rubber, said agent containing cadmium stearate as its essential active ingredient.

MARTIN LEATHERMAN.